

1

3,166,508  
**HYDROCARBON OILS OF REDUCED  
FOAMING PROPERTIES**

Joseph E. Fields, Ballwin, Mo., assignor to Monsanto  
Company, a corporation of Delaware  
No Drawing. Filed Jan. 16, 1963, Ser. No. 251,717  
16 Claims. (Cl. 252—51.5)

This invention provides hydrocarbon oils which are rendered antifoaming by the incorporation therein of certain polymeric acrylates.

In recent years the foam suppression of hydrocarbon oils has become of major importance owing to new developments in engine construction and use of foam-inducing additives. Attempts to solve the problem by defoaming existing oils using mechanical or physical means, e.g., by submitting them to heat treatment, absorption or filtration have proved of but little value. The most practical solution to this problem has been achieved by the use of antifoam additives.

Additives are currently added to hydrocarbon oils for many purposes. Advantageously, in the art, the additive performs a specific task when incorporated into the oil. An anti-corrosive additive preferably affects only the corrosive properties of the oil; a detergative additive, only the detergative properties; an extreme-pressure resisting additive, only the pressure-resisting properties; a viscosity index improving agent, only the viscosity properties; and an antifoam agent, only the antifoaming properties. Hydrocarbon oils, e.g., lubricants and motor-fuels are custom-tailored to serve well-defined needs and it is only by the careful blending of additives having individual functions that a properly compounded oil can be arrived at and successively duplicated.

An object of the present invention is to provide a hydrocarbon oil product containing an additive which will reduce and even completely eliminate the foam susceptibility of the hydrocarbon oil without substantially modifying or altering other properties of the oil. Another object of the invention is the provision of an antifoam additive for hydrocarbon oils which is retained in said oil under diverse operating conditions and during long periods of storage. Still another object of the invention is the provision of an antifoam additive which will not react with other additives generally employed with said oils. A further object of the invention is the provision of such an additive from readily available raw materials.

I have found that these objects and others which will be hereinafter defined are provided by the present invention wherein there is added to hydrocarbon oil compositions for the purpose of suppressing the foaming tendency thereof, a small amount, less than 0.1% by weight based on the weight of said oil, sufficient to suppress said foaming tendency and insufficient to modify substantially the viscosity characteristics of the oil, of an alkyl acrylate polymer selected from the class consisting of (A) a normally fluid homopolymer of an alkyl acrylate having at least 3 but less than 7 carbon atoms in the alkyl radical, (B) a normally fluid copolymer of at least two different alkyl acrylates in which the alkyl radical has from 1 to 18 carbon atoms and in which the average number of carbon atoms in the alkyl radicals of the copolymer molecule is at least 3 but less than 7 on a molar basis and (C) a copolymer having the oil-solubility of (A) and containing at least 50% by weight of an alkyl acrylate in which the alkyl radical has from 1 to 18 carbon atoms with the balance being a compound other than said acrylate and copolymerizable with the acrylate.

By "normally fluid" is meant thinly liquid to highly viscous polymers, the term "fluid" being preferred by the art to "liquid" in describing a viscous substance. However, in general polymers employed herein will be liquid

2

and have molecular weights of less than 10,000, usually less than 8,000 or 6,900, and preferably less than 5,000, which are much lower molecular weights than those customarily employed to modify viscosity index of oils.

In the prior art, polymeric acrylates have been added to hydrocarbon oils for the purpose of increasing the viscosity index thereof, for promoting adhesion of the oils to cylinders, for thickening oils to greases, etc. The addition of acrylates to oils in order to bring about modification of the viscosity, thickening or adhesive properties of the oil required at least 0.1% and up to about 5% of the acrylate polymer based on the weight of the oil composition. While the use of such proportions of the acrylates was effective in bringing about the desired changes, it was instrumental in increasing the foam susceptibility of the oil to such an extent that it required the addition also of foam suppressing additives to the oils. This is brought out in the Fenske et al. U.S. Patent No. 2,407,954, wherein esters of polyhydric alcohols and long chain fatty acids are added to hydrocarbon oils containing polymeric acrylates in quantities sufficient to improve the lubricating properties of the oil, said esters being added to such polymer-containing oils for the purpose of suppressing the foaming tendencies thereof. The suppression of foaming and emulsifying tendencies of hydrocarbon oils containing from 0.1% to 5% of polymeric acrylates also forms the subject of U.S. Patents Nos. 2,486,493 and 2,489,671 to Revukas wherein certain amino compounds or certain organic phosphorus compounds are used for this purpose.

In view of the fact that alkyl acrylate polymers have been reported to increase the foam susceptibility when added to hydrocarbon oils in amounts from 0.1% and upwards, it is surprising that when the particular alkyl acrylate polymers specified herein are added to the same oils in the lower proportions, i.e., in specified quantities less than 0.1% they serve as foam suppressors for the oils.

Normally fluid alkyl acrylate homopolymers which I have found to be effective in suppressing the foaming tendency of hydrocarbon oils when added thereto in a quantity of less than 0.06% by weight, based on the weight of the oil composition, are those polymers in which the alkyl chain length has from 3 to 6 carbon atoms. Polymeric methyl acrylate and polymeric ethyl acrylate are too oil-insoluble for the present purposes. Polymeric propyl acrylate provides a degree of oil-solubility which renders it effective as an antifoam agent, although its maximum antifoaming effect does not appear at a concentration which is as low as that at which the maximum antifoaming effect of polymeric butyl acrylate and polymeric amyl acrylate is found. For example, while polymeric butyl acrylate completely suppresses the foaming of a certain hydrocarbon oil composition at a concentration of as little as say, 1 to 5 parts per million, polymeric propyl acrylate must be employed in concentrations of as high as say, about 50 parts per million before the foaming tendency of the same oil composition is completely suppressed. Polymeric hexyl acrylate possesses foam suppressing effect but here, also, the concentrations at which it is useful differs from the concentrations at which polymeric amyl acrylate is useful, a greater quantity of this polymer being required to give the same effect. As is known in the art, the oil-solubility property of the polymeric alkyl acrylates changes with a change in the number of carbon atoms in the alkyl radical. I have found that the antifoaming effect of alkyl acrylate polymers also varies with the oil-solubility of such polymers.

The oil-solubility of homopolymeric alkyl acrylates having from 3 to 6 carbon atoms in the alkyl radical is such that a pronounced antifoam effect is demonstrated when

such polymers are added to hydrocarbon oil compositions at concentrations of less than 0.1%. A higher member, i.e., polymeric n-octyl acrylate or 2-ethylhexyl acrylate is too oil-soluble, and the next lower member, i.e., polymeric ethyl acrylate, is too oil-insoluble to possess antifoaming activity.

Acrylate-acrylate copolymers having the oil-solubility of homopolymeric acrylates may be obtained from mixtures of the lower alkyl acrylates, i.e., ethyl or methyl, and the higher alkyl esters such as n-octyl or dodecyl, provided that the average of the number of carbon atoms in the alkyl radicals of the ester mixture, based on molar proportions is at least 3, but less than 7, e.g., a copolymer made from a 70:30 mixture of methyl acrylate and n-propyl acrylate has a carbon chain average of 1.6 and is not useful for the present purpose, whereas a copolymer made from a 70:30 mixture of ethyl acrylate and 2-ethylhexyl acrylate has an average number of 6.2 carbon atoms in the total alkyl groups of the copolymer, and is a very effective antifoam agent. The average alkyl chain length in the copolymer molecule is extremely critical. The following table illustrates monomeric mixtures which when subjected to polymerizing conditions yield normally fluid antifoaming copolymers having an average chain length of from 3 to less than 7 carbon atoms on a molar basis:

| Lower Alkyl Acrylate | Mole Percent | Higher Alkyl Acrylate | Mole Percent | Av. No. Carbon Atoms In Total Alkyl Group of Copolymer, Molar Basis |
|----------------------|--------------|-----------------------|--------------|---------------------------------------------------------------------|
| Methyl acrylate      | 50           | Nonyl                 | 50           | 5.0                                                                 |
| Do                   | 40           | Decyl                 | 60           | 6.4                                                                 |
| Do                   | 30           | Octyl                 | 70           | 5.9                                                                 |
| Do                   | 60           | 2-ethylhexyl          | 40           | 3.8                                                                 |
| Do                   | 10           | n-Amyl                | 90           | 4.6                                                                 |
| Do                   | 5            | n-Butyl               | 95           | 3.85                                                                |
| Do                   | 63           | Dodecyl               | 37           | 5.07                                                                |
| Ethyl acrylate       | 30           | 2-ethylhexyl          | 70           | 6.2                                                                 |
| Do                   | 50           | Decyl                 | 50           | 6.0                                                                 |
| Do                   | 60           | Undecyl               | 40           | 5.6                                                                 |
| Do                   | 20           | Isoamyl               | 80           | 4.4                                                                 |
| Do                   | 18           | n-Butyl               | 82           | 3.64                                                                |

It is preferred to employ alkyl acrylate polymers having an average alkyl chain length of 4 to 6.5 carbon atoms, rather than the broader range of 3 to 7 carbon atoms; a still more preferred range is that of 4.5 to 6 carbon atoms. As is known to those skilled in the art more than two different alkyl acrylates may be polymerized together to give copolymers having an average of at least 3 but less than 7 carbon atoms in the total alkyl groups of the copolymer. Thus, there may be used a mixture consisting of 50 mole percent of methyl acrylate, 25 mole percent of dodecyl acrylate and 25 mole percent of hexyl acrylate to yield a copolymer having a total of 5.0 carbon atoms in the alkyl groups thereof. Copolymers containing a plurality of alkyl acrylates having from 1 to 18 carbon atoms in the alkyl radicals may be prepared from mixtures containing the various acrylates in molar proportions calculated to give an average of at least 3 but less than 7 carbon atoms in the total alkyl radicals of the copolymer.

Just as the oil-solubility of the acrylate-acrylate copolymers may be controlled by appropriate selection of the monomeric acrylates which are to be copolymerized and the maximum foam-suppressing power thus readily arrived at, it may also be pointed out that the same result may be achieved by preparing copolymers of alkyl acrylates with other monomers which are copolymerizable therewith. In general, the weight proportion of the alkyl acrylate content of these copolymers should be at least 50%. The general principles to be employed in combining monomers in order to obtain effective antifoaming properties when dissolved in any hydrocarbon oil are as follows:

Methyl and ethyl acrylate homopolymers as has already been pointed out are generally too oil-insoluble to

impart anti-foaming properties. On the other hand, such monomers as alkylated styrene, the higher alkyl (5 to 18 carbon atoms) methacrylates, the higher alkyl maleates or fumarates and vinyl esters of the higher aliphatic mono-carboxylic acids are useful with the above-mentioned lower alkyl acrylates to give copolymers having the desired degree of solubility.

When the alkyl acrylate component is one having an alkyl radical of from 8 to 18 carbon atoms, the co-monomer selected should be one which in the homopolymeric form possesses little or no oil-solubility. Examples of these insolubility-promoting monomers are: acrylonitrile, methacrylonitrile, the lower alkyl methacrylates such as methyl, ethyl or propyl methacrylates, the lower vinyl esters such as vinyl acetate or vinyl propionate and the lower alkyl maleates, fumarates, or itaconates, such as for example, the methyl or ethyl esters thereof.

That the oil solubility of polymers can be regulated by selecting monomers whose homopolymers have varying oil solubilities is generally recognized in the art. Thus, according to Port et al. (Ind. Eng. Chem. 43, 2106-7 (1951)):

"If two monomers are available and the homopolymer of one is highly soluble and that of the other is insoluble in petroleum oils, then the copolymers should be expected to have a graded solubility."

Also, in the Tutwiler Patent No. 2,637,698, there are prepared copolymers having a desired degree of oil solubility by polymerizing a mixture of an alkyl acrylate having from 8 to 24 carbon atoms in the alkyl radical and an alkyl itaconate having from 1 to 4 carbon atoms in the alkyl radical. Tutwiler states:

"The oil solubility of the finished copolymeric material is governed to a considerable extent by the ratio of the alpha methylene dicarboxylic esters, which supply short side chains to the copolymer, to the alpha, beta unsaturated monocarboxy esters, which supply long side chains to the copolymer, employed in the copolymerization reaction."

For some purposes extremely oil-soluble polymers are desired for incorporation into the oil. This is particularly true when oils have a high paraffin content. For such oils the oil solubility of even the higher alkyl acrylates is increased by copolymerization with a nuclearly alkylated styrene, the homopolymers of which are likewise very oil soluble. Such increase of oil solubility is shown in the Gleason U.S. Patent No. 2,366,517 and the Harrison U.S. Patent No. 2,593,444. Styrene or a nuclearly alkylated styrene may also be employed with a lower alkyl acrylate such as ethyl or methyl acrylate, whereby there are obtained copolymers of moderate solubility. Very highly oil soluble acrylate copolymers have also been prepared by polymerizing a mixture of a higher alkyl acrylate and a higher vinyl ester such as vinyl laurate, as in the Van Horne et al. U.S. Patents Nos. 2,600-450-1. While the vinyl esters generally give homopolymers of low solubility the lower esters being practically oil-insoluble, vinyl esters in which the acid portion contains from 6 to 12 carbon atoms give homopolymers whose oil solubility increases with the carbon content of the monomer, so that the degree of solubility of the acrylate-vinyl ester copolymer is a function of the alkyl chain length of each of the two esters and the proportion of the insolubilizing:solubilizing monomer used. In the Dittmar et al. U.S. Patent No. 2,232,595 the solubility of acrylate polymers in paraffin wax is also regulated by alkyl chain length of the acrylate as well as by the nature of the copolymerizing monomer, if any.

Variation in solubility of a copolymer to fit individual requirements is a commonly employed procedure in the art. Concerning present day practices in this respect Spurlin (J. Polymer Science 3, 734 (1948)) makes these remarks about altering a polymer to secure a desired degree of solubility:

"If it is desirable to work with polymer solutions for

either commercial or scientific purposes, it is frequently more desirable to alter the polymer for the best balance of solubility and physical properties than to go to great effort to use an available material. Manufacturers have long been conscious of this, and customarily supply materials tailored to fit individual application. Because of the wide variation of solubility characteristics that is deliberately introduced by the manufacture of copolymers and cellulose derivatives, it is usually wise to consult the manufacturer's literature for detailed solubility characteristics."

Numerous examples of useful copolymers having the oil solubility of homopolymers of alkyl acrylates having 3 to 6 carbon atoms will be given; and since tailoring of copolymers for the purpose of conferring thereto certain solubility characteristics is an established practice in the art, formulation of other alkyl acrylate copolymers having the desired degree of oil-solubility will present no problem to those skilled in the art.

The presently useful alkyl acrylate polymers may be prepared by methods generally known to the art. The polymerization may be effected in mass, emulsion or solution in the presence of a free-radical liberating agent as catalyst and in the presence or absence of known polymerization regulators. When effected in mass, the monomer, or mixture of monomers, is simply maintained in the presence of the free-radical liberating agent, advantageously with agitation, and at temperatures of from, say, 35° C. to 130° C. until the polymerization is substantially completed. When the polymers are formed by emulsion polymerization methods, an emulsion of the monomer components is made in an aqueous solution using suitable emulsifying agents such as soap or an alkyl-substituted sulfosuccinate, and the emulsion is then subjected to a polymerizing temperature which may vary from 25° C. up to the boiling point of water.

In solution polymerization, the monomer or monomers are dissolved in an inert liquid, and the resulting solution is agitated, preferably in the presence of a polymerizing catalyst at temperatures of from 25° C. to the boiling point of the solution to effect copolymerization of said mixture. Solvents which may be employed are generally substantially neutral organic liquid media, e.g., aliphatic, aromatic alkyl aromatic or alicyclic hydrocarbons such as hexane, benzene, ethylbenzene or cyclohexane; ketones such as methyl ethyl ketone or acetone, esters such as ethyl acetate or methyl propionate; chlorinated hydrocarbons such as carbon tetrachloride or chloroform; ethers such as ethyl ether or dioxane. Since the polymers are used as oil additives, it is advantageous to effect the polymerization in a solvent which has no deleterious effect on the hydrocarbon oil to be treated, so that the resulting solutions of polymer may be added directly to said oil without first having to separate the polymer from the reaction media.

The presently useful alkyl acrylate polymers are very advantageously prepared by conducting the polymerization in the presence of polymerization modifiers, whereby the solubility of the polymers may be further regulated. As modifiers there may be used such well-known "chain-transfer agents," "telomerizers" or "regulators" as the alkyl mercaptans, e.g., tert-butyl mercaptan or n-dodecyl mercaptan; the polyhaloalkanes such as carbon tetrachloride, chloroform or bromoform; the nitroalkanes such as nitroethane or 2-nitropropane; liquid hydrocarbons such as toluene, ethylbenzene, or kerosene, etc. The chain terminating agent may be used as a solvent during the reaction or it may be incorporated with an extraneous solvent, e.g., dioxane, acetone, paraffin hydrocarbons, etc.

The generally known polymerizing catalysts may be employed in preparing the polymers. There may be used, for example, such organic peroxidic compounds as acetyl, benzoyl, lauroyl or stearoyl peroxide and tert-butyl or cumene hydroperoxide; inorganic per-compounds such as hydrogen peroxide, sodium perborate, or potas-

sium persulfate, diazo compounds such as azo-bis-isobutyronitrile, alpha, alpha'-azodiisobutyramide, etc.

The preparation of the useful polymers may also be carried out without the use of catalysts, e.g., by thermal polymerization.

The polymerization reaction may be effected batchwise, e.g., by agitating the solutions at increased temperatures, say at 80-110° C., until reaction has been completed, or continuously, i.e., by constantly removing the polymer 10 while replenishing one or both of the monomers and/or catalyst and regulating agent. When operating batchwise, the reaction product, i.e., the polymer may be separated from the reaction mixture by distilling off the solvent and any unreacted starting material; however in 15 practice, separation of the polymer is not generally necessary. Instead, the reaction mixture, comprising a solution of the polymer in the solvent, may be used directly as the antifoaming additive.

The present polymers are effective antifoaming agents 20 when they are employed in very low proportions, i.e., in amounts of less than 0.06 percent by weight, based on the weight of the total hydrocarbon oil composition. From .001 percent to .01 percent of the polymers is preferred, but may be varied depending upon the nature of 25 the oil, amounts less than 0.04 percent by weight usually being sufficient. Heavy oils and oils containing foam-inducing adjuvants require more of the polymers than do base oils with lesser foaming characteristics.

The antifoaming effect of the present acrylate polymers 30 is not materially affected by the presence of other adjuvants in the oil. Since the acrylate polymers are present in the oils in oily very small quantities, the use of even very acidic or very basic adjuvants in the oil has substantially no effect on the antifoam additives. Hydrocarbon oils containing the present antifoaming agents are stable when stored over long periods of time and also when subjected to heat and pressures representative of conditions encountered under operating conditions.

Hydrocarbon oils which are rendered substantially anti- 35 foaming by incorporation therein of quantities of less than 0.06 percent of the present polymers are synthetic or petroleum stocks of varying viscosities such as lubricating oils for internal combustion engines and motors, diesel fuels and lubricants and pressure transfer media, e.g., industrial lubricants, process oils, hydraulic oils, turbine oils, cutting oils, fluid greases, gear oils, shock absorber oils, spindle oils, journal bearing oils, pneumatic tool lubricants, etc. They may be synthetic or natural hydrocarbons of any type, i.e., paraffinic, naphthenic, aromatic or blended.

Of particular interest is the usefulness of the present 40 normally fluid acrylate polymers as antifoaming agents for lubricating compositions containing foam-inducing additives. As will be shown hereinafter, the present polymers 45 retard foaming of lubricating oils containing additives which ordinarily tend to increase the foam-susceptibility of base oils. Thus, the acrylate polymers function very efficiently as antifoaming agents for hydrocarbon lubricants containing detergents and pour-point depressants 50 generally, and particularly such detergents as the metal salts of aliphatic, cyclo-aliphatic, aromatic and aromatic-aliphatic compounds containing as substituents at least one salt-forming radical, and a hydrocarbon chain of at least 4 carbon atoms. The structure and efficiency 55 of some of such additives are described on pages 169-176 of the book *Motor Oils and Engine Lubrication*, by Carl W. Georgi, published by Reinhold Publishing Corporation, New York, 1950. As illustrations of such detergent additives may be mentioned aluminum, calcium or lithium 60 hexadecylphenate, the barium or magnesium salt of sulfated dodecylphenol, the magnesium or strontium salt of an alkyl substituted naphthol in which the alkyl substituent is derived from wax, the barium salt of oleyl ester of carbonic acid; barium cetyl phthalate, the calcium 65 salt of wax-substituted phenoxyphenol, the barium of wax-

70 75

substituted, sulphated hydroxydiphenyl sulfide, etc. The present acrylates may also be used as foam-suppressing additives for oils containing deterutive additives such as the wax-substituted benzene sulfonates, the petroleum sulfonates, or salts of alkylhydroxyphenyl sulfides.

The present acrylate polymers are also efficient anti-foaming agents for lubricant compositions containing extreme-pressure additives, such as the aromatic and alkyl-

time any unreacted material was removed by distilling through a 10" Vigreux column. The residues were low-molecular weight polymers. The average molecular weights given below were based on halogen content of the polymer determined by chemical analysis. The following preparations were tested for defoaming action in 200 cc. of Champlin 30 base oil, employing the testing procedure described above.

| Polymer                                                                                                                                         | Foam, cc. at 5 Min. (Polymer in p.p.m.) |     |     |     |     |     |
|-------------------------------------------------------------------------------------------------------------------------------------------------|-----------------------------------------|-----|-----|-----|-----|-----|
|                                                                                                                                                 | None<br>710-720                         | 50  | 10  | 5   | 2   | 1   |
| From .3M Et acrylate, .73g. Bz <sub>2</sub> O <sub>2</sub> , & .6M CCl <sub>4</sub> ; 34.4g. polymer, 9.24% Cl, M.W. 1535.                      |                                         | 705 |     |     |     |     |
| From .263M Pr acrylate, .6g. Bz <sub>2</sub> O <sub>2</sub> , 1M CCl <sub>4</sub> ; 31g. polymer, 2.99% Cl, M.W. 4750.                          |                                         | 10  | 245 |     |     |     |
| From 2M Bu acrylate, 6.5g. Bz <sub>2</sub> O <sub>2</sub> , 10M CCl <sub>4</sub> ; 510g. polymer, 3.58% Cl, M.W. 3950.                          |                                         |     | 10  | 165 | 420 |     |
| From 2M Bu acrylate, 7.5 cc. of 75% Cumene hydroperoxide, 10M CCl <sub>4</sub> ; 220g. polymer, 2.13% Cl, M.W. 6650.                            |                                         |     | 0   | 0   | 20  |     |
| From .3M Bu acrylate, .6M CCl <sub>4</sub> , .872g. Bz <sub>2</sub> O <sub>2</sub> ; 37.1g. polymer, 2.65% Cl, M.W. 5350.                       |                                         | 0   | 10  | 30  | 270 |     |
| From .3M Bu acrylate, .9M CHCl <sub>3</sub> , 1.94g. Cumene hydroperoxide; 39.2g. polymer, 1.59% Cl, M.W. 6690.                                 |                                         |     | 0   | 0   | 65  |     |
| From 2M Bu acrylate, 154g. CCl <sub>4</sub> , 1.5g. Bz <sub>2</sub> O <sub>2</sub> ; 32g. polymer, 3.98% Cl, M.W. 3560.                         |                                         |     | 55  |     |     |     |
| From 2M Bu acrylate, 10M CHCl <sub>3</sub> , 6.5g. Bz <sub>2</sub> O <sub>2</sub> ; 505g. polymer, 2.08% Cl, M.W. 5130.                         |                                         |     | 0   | 0   | 20  |     |
| From 8M Bu acrylate, 40M CHCl <sub>3</sub> , 20.5g. Bz <sub>2</sub> O <sub>2</sub> ; 982g. polymer, M.W. 5330.                                  |                                         |     | 0   | 10  | 100 |     |
| From 30g. Amyl acrylate 119g. CHCl <sub>3</sub> , .6g. Bz <sub>2</sub> O <sub>2</sub> ; 28g. polymer, M.W. 5700.                                |                                         | 0   | 0   | 0   | 20  |     |
| From .211M Am acrylate, 1.5g. Bz <sub>2</sub> O <sub>2</sub> , 1M CCl <sub>4</sub> ; 31g. polymer, 4.6% Cl, M.W. 3100 <sup>1</sup> .            |                                         |     |     | 0   | 10  | 140 |
| From .211M Am acrylate, .6g. Bz <sub>2</sub> O <sub>2</sub> , 1M CCl <sub>4</sub> ; 30.3g. polymer, 3.12% Cl, M.W. 4550.                        |                                         | 0   | 0   | 0   | 10  | 85  |
| From .193M hexyl acrylate, .6g. Bz <sub>2</sub> O <sub>2</sub> , 1M CCl <sub>4</sub> ; 27.5g. polymer, 2.85% Cl, M.W. 4980.                     |                                         | 0   | 133 |     |     |     |
| From 2M 2-ethylhexyl acrylate, .6M CCl <sub>4</sub> , 1.84g. Bz <sub>2</sub> O <sub>2</sub> ; 37.1g. polymer, 2.4% Cl, M.W. 5765 <sup>1</sup> . |                                         | 780 |     |     |     |     |

<sup>1</sup> Reaction time 4 days instead of 48 hours.

aromatic compounds of from 5 to 30 carbon atoms which contain a thiocarbonate group, e.g., chlorododecyl ethyl xanthate or chlorobenzyl methyl xanthate; sulfocarbonates such as trichlorobenzyl ethyl sulfocarbonate; trithiocarbonates such as (dichlorophenyl) ethyl propyl trithiocarbonate; dithiocarbonates such as tetrachlorohexyl-p-tolyl dithiocarbonate; and thiocarbonates such as hexachlorotricosyl butyl thiocarbonate. Of the above, the xanthates generally have an economic advantage.

The present active defoaming compounds may be employed with compounded oils generally, such as hydrocarbon oils containing additives such as viscosity index improvers, pour-point depressants, metal deactivators, antioxidants, or extreme pressure agents, e.g., with phosphate-containing gear oils, corrosion-inhibited turbine oils, etc.

The present invention is further illustrated, but not limited, by the following examples:

#### Example 1

The effectiveness of antifoaming additives in hydrocarbon oils may be determined according to the procedure generally described in Designation L-12-445 of the Co-ordinating Lubricants Research Committee of the Co-ordinating Research Council, New York. Briefly this procedure involves bubbling air or an inert gas such as nitrogen through the hydrocarbon oil to be tested employing standard apparatus and standard conditions and reading the volume of foam produced.

A series of liquid polymeric alkyl acrylates was prepared as follows:

The alkyl acrylate was mixed with the halomethane indicated in the table below and the catalyst in the proportions shown below, and bottles of the respective mixtures were maintained on a rotating rack at a temperature of from 90-95° C. for 48 hours. At the end of that

The above results show that while the antifoaming effect of the polymeric alkyl acrylates varies somewhat with the nature of the alkyl radical and with the average molecular weight of the polymer, good antifoaming activity is obtained with the polymeric propyl, butyl, amyl and hexyl acrylates at even very low concentrations, i.e., at 50 parts of the polymer per million parts by weight of the oil (0.005% by weight). Within the concentration range of from one to 50 parts per million (0.0001% to 0.005%) the amyl acrylate polymer provides the optimum antifoaming activity. However, economy does not require these very low concentrations. Thus, the more readily available polymeric propyl acrylate which is not so active at the very low concentrations but which nevertheless possesses very good foaming efficiency at concentrations between 0.005% and 0.06% may often be employed more advantageously as the antifoaming agent than the extremely active polymeric amyl acrylate.

#### Example 2

This example shows the antifoaming effect of various polymeric butyl acrylates on three different oils. The testing procedure was substantially that employed in Example 1, except that it was performed with smaller samples, i.e., instead of using 200 cc. of the oil as in Example 1, there was used 30 ml. of oil.

In the following table the three different oils used are denoted as follows:

- (1) Mid-Continent solvent refined SAE 30.
- (2) Mid-Continent solvent refined SAE 10.
- (3) Champlin SAE 30.

Under the test conditions each of these base oils gave a heavy foam in the absence of the antifoaming polymers. In the presence of the indicated polymers at 50 p.p.m.

concentration the results shown in the following table were obtained:

as catalyst. The results obtained are shown in the following table.

| Polymer Additive Used | Amt. of Tert. C <sub>4</sub> H <sub>9</sub> SH |         | Percent S In Polymer | Foam (cc.) at 5 Min. (Additive in p.p.m.) |     |     |       |       |       |  |
|-----------------------|------------------------------------------------|---------|----------------------|-------------------------------------------|-----|-----|-------|-------|-------|--|
|                       | Acrylate                                       |         |                      | None<br>710-720                           | 50  | 20  | 10    | 5     | 2     |  |
|                       | G.                                             | Percent |                      |                                           |     |     |       |       |       |  |
| Butyl                 | 3.0                                            | 10.0    | 1.79                 | 60                                        | 415 | 645 | ----- | ----- | ----- |  |
| Do.                   | 1.5                                            | 5.0     | 0.91                 | 0                                         | 0   | 265 | ----- | ----- | ----- |  |
| Do.                   | 0.6                                            | 2.0     | 0.29                 | 10                                        | 155 | 375 | 20    | 165   | 20    |  |
| Do.                   | 0.3                                            | 1.0     | 0.16                 | 0                                         | 20  | 10  | 43    | 250   | 95    |  |
| Do.                   | 0.15                                           | 0.5     | 0.05                 | 10                                        | 25  | 0   | 0     | 20    | 30    |  |
| Do.                   | 0.06                                           | 0.2     | 0.02                 | 10                                        | 25  | 0   | 0     | 20    | 30    |  |
| Amyl                  | 0.3                                            | 1.0     | 0.25                 | 10                                        | 25  | 0   | 0     | 20    | 30    |  |
| Do.                   | 0.15                                           | 0.5     | 0.12                 | 10                                        | 25  | 0   | 0     | 20    | 30    |  |
| Do.                   | 0.06                                           | 0.2     | 0.02                 | 10                                        | 25  | 0   | 0     | 20    | 30    |  |

| Polymer                                         | Molecular Weight | Base Oil | Results  |
|-------------------------------------------------|------------------|----------|----------|
| Butylacrylate (prepared in CCl <sub>4</sub> )   | 2,000            | 1        | No foam. |
| Do.                                             | 3,528            | 2        | Do.      |
| Do.                                             | 4,807            | 2        | Do.      |
| Do.                                             | 5,011            | 1        | Do.      |
| Do.                                             | 5,352            | 1        | Do.      |
| Butyl acrylate (prepared in CHCl <sub>3</sub> ) | 1,513            | 1        | Do.      |
| Do.                                             | 3,253            | 2 & 3    | Do.      |
| Do.                                             | 4,565            | 2 & 1    | Do.      |
| Do.                                             | 5,266            | 2 & 3    | Do.      |
| Do.                                             | 6,690            | 1        | Do.      |
| Butyl acrylate (prepared in CHBr <sub>3</sub> ) | 2,899            | 1        | Do.      |
| Do.                                             | 3,316            | 2        | Do.      |

### Example 3

Stability of various halomethane chain-terminated polymeric alkyl acrylates in Champlin 30 oil under conditions of ordinary storage was determined by storing for 15 days at room temperature samples of oil containing the respective polymers and then submitting the stored samples to the antifoaming test described in Example 1. No foaming was observed with samples containing 5 parts per million of the following polymers (see Example 1 for polymer preparation).

Butyl acrylate, CHCl<sub>3</sub> terminated. Mol Wt.=5130

Amyl acrylate, CCl<sub>4</sub> terminated. Mol Wt.=4550

Amyl acrylate, CHCl<sub>3</sub> terminated. Mol Wt.=5700

Similar results are obtained with oils containing not only the above antifoaming agents but also other lubricant additives, e.g., gear oils containing extreme pressure adjuvants, etc.

### Example 4

Employing the testing procedure described in Example 1 there was determined the antifoaming effect of some mercaptan-terminated, polymeric butyl and amyl acrylates when employed in concentrations of from 2 parts to 50 parts of the polymer per million parts of Champlin 30 oil. The polymers employed were prepared by heating for 48 hours at 90-95° C., thirty grams of the indicated acrylate and the indicated quantities of tert.-butyl mercaptan in benzene solution and in the presence of benzoyl peroxide

The above results show that while the antifoaming effect of the mercaptan-terminated polymeric alkyl acrylates varies with the quantity of mercaptan employed and thus with the average molecular weight of the polymer, as indicated by sulfur-content, good antifoaming activity is obtained with the polymers at even very low concentrations, i.e., at less than 50 parts of the polymer per million parts by weight of the oil (less than 0.005% by weight). At the concentrations of less than 20 parts per million (0.002%) polymers having a sulfur content of less than 1.0% provide the optimum antifoam activity.

### Example 5

Stability of various mercaptan-terminated polymeric alkyl acrylates in Champlin 30 oil under conditions of ordinary storage was determined by storing for 15 days at room temperature samples of oil containing the respective polymers and then submitting the stored samples to the antifoaming test described in Example 1. No foaming was observed with samples containing 5 parts per million of the following polymers:

Polymeric butyl acrylate, terminated with tert.-dodecyl mercaptan, and containing 0.38% sulfur.

Polymeric butyl acrylate, terminated with tert.-butyl mercaptan, and containing 0.16% sulfur.

Polymeric amyl acrylate, terminated with tert.-butyl mercaptan, and containing 0.12% sulfur.

### Example 6

Employing the testing procedure described above there was determined the antifoaming effect of polymeric butyl or amyl acrylates, prepared in toluene, when employed in concentrations of from 2 parts to 10 parts of the polymer per million parts of a Champlin 30 base oil. The polymers employed were prepared by heating for 48 hours at 90-95° C. the indicated acrylate in toluene in the proportions shown below, and in the presence of benzoyl peroxide as catalyst. The viscosities shown below are 10% cyclohexanone specific viscosities at 25° C. The results obtained are shown in the following table:

| Polymer Additive Used | Toluene |     | Bz <sub>2</sub> O <sub>2</sub><br>g. | Specific<br>Viscosity<br>of Polymer | Foam (cc.) at 5 Min.<br>(Additive in p.p.m.) |    |     |     |  |  |
|-----------------------|---------|-----|--------------------------------------|-------------------------------------|----------------------------------------------|----|-----|-----|--|--|
|                       | Alkyl   |     |                                      |                                     | None<br>710-720                              | 10 | 5   | 2   |  |  |
|                       | G.      | G.  |                                      |                                     |                                              |    |     |     |  |  |
| Butyl                 | 30      | 108 | 1.5                                  | 1.65                                | 0                                            | 5  | 205 | 205 |  |  |
| Do.                   | 100     | 333 | 1.0                                  | -----                               | 0                                            | 0  | 25  | 25  |  |  |
| Do.                   | 100     | 333 | 1.19                                 | 1.30                                | 0                                            | 0  | 20  | 10  |  |  |
| Do.                   | 100     | 333 | 2.20                                 | -----                               | 0                                            | 0  | 30  | 30  |  |  |
| Do.                   | 100     | 333 | 0.6                                  | 1.43                                | 0                                            | 0  | 15  | 15  |  |  |
| Amyl                  | 30      | 100 | 0.6                                  | 2.13                                | 0                                            | 10 | 60  | 60  |  |  |
| Do.                   | 30      | 100 | 0.3                                  | -----                               | 0                                            | 0  | 20  | 20  |  |  |
| Do.                   | 30      | 108 | 0.6                                  | 2.18                                | 0                                            | 0  | 20  | 20  |  |  |

<sup>1</sup> Cumene hydroperoxide employed instead of benzoyl peroxide.

<sup>2</sup> 1 g. of cumene hydroperoxide and 1 g. of benzoyl peroxide.

## 11

The above results show that good antifoaming activity is obtained with the polymers at very low concentrations, i.e., at less than 10 parts of the polymer per million parts by weight of the oil (less than 0.001% by weight).

## Example 7

Stability of the various liquid alkyl acrylate polymers of Example 6 in Champlin 30 oil under conditions of ordinary storage was determined by storing for 15 days at room temperature samples of oil containing the respective polymers and then submitting the stored samples to the antifoaming test described in Example 1. No foaming was observed with samples containing 5 parts per million of the following polymers from Example 6:

Polymeric butyl acrylate, specific viscosity = 1.65.

Polymeric amyl acrylate, specific viscosity = 2.13.

## Example 8

Butyl and amyl acrylate were polymerized while dissolved in benzene. Reaction mixtures comprising 30 g. of either butyl or amyl acrylate, 92 g. of benzene and 0.3 g. of benzoyl peroxide were heated for 48 hours at 90° C. Removal of unreacted solvent and monomer gave 29.5 g. of a polymer in the case of butyl acrylate and 28 g. of a polymer in the case of amyl acrylate. Additive concentrates consisting of 2 g. of the polymer dissolved in 18 cc. of mineral spirits were prepared and added to Champlin SAE 30 oil. Employing the testing procedure of Example 1, the following results were obtained:

| Polymer        | Foam (ml.), after 5 Min.<br>(Additive in p.p.m.) |    |    |    |     |
|----------------|--------------------------------------------------|----|----|----|-----|
|                | None 715                                         | 20 | 10 | 5  | 2   |
| Butyl acrylate |                                                  |    | 10 | 20 | 200 |
| Amyl acrylate  |                                                  | 10 | 0  |    | 20  |

## Example 9

Butyl or amyl acrylate was polymerized while dissolved in Stoddard solvent (a petroleum distillate). Reaction was effected by maintaining bottles of the reactants on a rotating rack (43 r.p.m.) for 48 hours at a temperature of 85–90° C. Each reaction mixture consisted of 30 g. of the acrylate, 100 g. of Stoddard solvent and 0.3 g. of benzoyl peroxide. In one instance, shown below, tert-butyl mercaptan was also present. The polymers were not isolated from the reaction mixture; instead, each reaction mixture was diluted with additional Stoddard solvent to 244 g., and the diluted material was employed as the antifoam additive for Champlin SAE 30 oil. Assuming complete polymerization of the monomers, each solution was taken to be a 12.3 percent by weight concentrate of the polymeric acrylate. Employing the testing procedure of Example 1, the following results were obtained with the respective polymer solutions:

| Polymer                     | Foam (ml.) at 5 Min.<br>(Polymer in p.p.m.) |    |    |    |
|-----------------------------|---------------------------------------------|----|----|----|
|                             | None 715                                    | 10 | 5  | 2  |
| Butyl acrylate              |                                             | 0  | 0  | 20 |
| Butyl acrylate <sup>1</sup> |                                             | 0  | 0  | 20 |
| Amyl acrylate               |                                             | 0  | 10 | 50 |

<sup>1</sup> Also present, 1.0% tert-butyl mercaptan, based on weight of monomer.

## Example 10

A mixture consisting of 256 g. (2 moles, 284 cc.) of butyl acrylate, 1540 g. (10 moles, 965 cc.) of carbon tetrachloride and 14.25 g. of 72 percent cumene hydroperoxide (4 percent by weight of pure hydroperoxide based on the acrylate) was charged to 8 small bottles (160 cc. each). These were maintained at 95° C. for 42

## 12

hours. The reaction mixtures were then combined and the whole was stripped to yield 202 g. of the substantially pure polymeric butyl acrylate. In order to prepare an antifoam concentrate, 100 g. of the stripped product was dissolved in 300 g. of kerosene and then further diluted to 20 percent solids by the addition of 100 g. of toluene. The resulting concentrate was then added to aircraft engine oil 120 in a quantity to give 10 parts of polymer per million parts of oil, and the foam susceptibility of the resulting oil was determined as described in Example 1, except that instead of using 200 cc. of oil, 40 cc. of the oil was employed for the test. No foam was obtained at the 10 p.p.m. concentration (0.001 percent) whereas the untreated oil gave 70 cc. of foam under the same test conditions.

## Example 11

Into a flask equipped with stirrer and thermometer there was placed 225 g. of butyl acrylate and 750 g. (865 cc.) of toluene. The reaction mixture was brought to a temperature of 100° C. within 35 minutes and there was initiated the portionwise addition of a catalyst solution consisting of 6.25 g. (7.3 cc.) of commercial 72 percent cumene hydroperoxide diluted with toluene to 25 cc. The first portion added was 5 cc.; the remaining 20 cc. was added in 2-cc. portions at intervals during the subsequent 3.2 hours, during which period the pot temperature was maintained at about 110° C. Heating at 109.0°–109.5° C. was continued for an additional 3 hours, at which time polymerization was substantially completed. Refractive index determinations on samples of the reaction mixture withdrawn at intervals during the run showed 55 percent polymerization after 1.25 hours and 79 percent after 2 hours.

The reaction mixture was then stripped at a maximum pot temperature of 200° C./2 mm. to give as a residue 215 g. of the viscous, liquid polymer. In order to prepare an antifoam concentrate, 100 g. of the polymer was added to 300 g. of kerosene and 100 g. of toluene. This gave a concentrate having 20 percent by weight of polymer. When tested with aircraft engine oil 120 as in Example 10, no foam was obtained at a concentration of 10 parts of polymer per million parts of oil.

## Example 12

For still another test with aircraft engine oil 120, amyl acrylate was prepared in carbon tetrachloride as follows: A mixture consisting of 480 g. of amyl acrylate, 2464 g. of carbon tetrachloride and 9.6 g. of benzoyl peroxide was charged to 16 bottles, and the bottles were tumbled for 40 hours at a temperature of 95° C. The contents of all were combined, and the combined material stripped at a maximum pot temperature of 160° C./3 mm. to give 475 g. of the viscous liquid polymer. When tested as in Example 10, the polymer rendered aircraft engine oil 120 non-foaming when incorporated therein at a concentration of 10 parts of polymer per million parts of oil. It was similarly efficient when tested with Champlin SAE 30 oil.

## Example 13

This example shows the effect of heat on the antifoaming effect of a polymeric amyl acrylate. The polymer was prepared by tumbling for 48 hours a mixture consisting of 30 g. of the acrylate, 154 g. of carbon tetrachloride, and 0.15 g. of benzoyl peroxide, and removing the solvent from the resulting reaction product. A Champlin 30 oil was incorporated with the additive to give a concentration of additive of ten parts per million, and the treated oil was tested for foaming substantially as described in Example 1, except that tests were made at the various temperatures shown below and that they were performed on a small scale, i.e., instead of using 200 cc. of oil, the volume of test sample plus bubbler was 35 cc.

The following results were obtained with the untreated and treated oils.

| Temperature, ° C. | Foam (cc.), at 5 Minutes |             |
|-------------------|--------------------------|-------------|
|                   | Untreated Oil            | Treated Oil |
| 25                | 100                      | 0           |
| 60                | 75                       | 0           |
| 75                | 60                       | 0           |
| 90                | 60                       | 10          |

*Example 14*

A Champlin SAE 30 oil was incorporated with 4% by weight of a detergent additive and samples of the compounded oil thus obtained were then admixed with various polymeric acrylates in concentrations of from 5 parts to 50 parts of the polymer per million parts of the detergent-containing oil. The detergent additive which was employed was a barium salt of an alkyl aromatic sulfonic acid in which the alkyl radical has from 22 to 30 carbon atoms and will be hereinafter designated as D-1. The polymers employed were prepared by heating the indicated alkyl acrylate for 48 hours at 90-95° C. in the presence of the indicated chain-terminating agent, e.g., an alkylbenzene, alkyl mercaptan or polyhalomethane and in the presence of benzoyl peroxide as catalyst. Samples of the oil containing 4% by weight of D-1, and the respective polymeric acrylates in the quantities shown below were submitted to the testing procedure described in Example 1 in order to determine the antifoaming effect of the polymers. The results obtained are shown in the following table:

| Polymer Additive                                                         | Foam (cc.) at 5 min. (Additive in p.p.m.) |    |         |         |       |
|--------------------------------------------------------------------------|-------------------------------------------|----|---------|---------|-------|
|                                                                          | None<br>780-765                           | 50 | 20      | 10      | 5     |
| Propyl acrylate, $CCl_4$ terminated, Mol Wt.=4,750                       |                                           | 10 | 550-575 | -----   | ----- |
| Butyl acrylate, $CCl_4$ terminated, Mol Wt.=5,352                        |                                           | 0  | 10      | 520-550 | ----- |
| Butyl acrylate, tert.-butyl mercaptan terminated, percent S=0.25         |                                           | 0  | 0       | 90      | 165   |
| Butyl acrylate, toluene terminated, specific viscosity=1.65 <sup>1</sup> |                                           | 0  | 0       | 20      | 80    |
| Butyl acrylate, $CHCl_3$ terminated, Mol Wt.=5,130                       |                                           | 0  | 0       | 10      | 20    |
| Amyl acrylate, $CCl_4$ terminated, Mol Wt.=4,550                         |                                           |    |         | 0       | 0     |
| Amyl acrylate, toluene terminated, Specific viscosity=2.13 <sup>1</sup>  |                                           |    |         | 0       | 0     |
| Amyl acrylate, tert.-butyl mercaptan terminated, percent S=0.12          |                                           |    |         | 0       | 0     |
| Hexyl acrylate, $CCl_4$ terminated, Mol Wt.=4,980                        |                                           | 0  | 105-110 | -----   | ----- |

<sup>1</sup> 10% cyclohexanone.

*Example 15*

Champlin 30 oil was heat-blended with 4% by weight of the detergent additive D-1 (see Example 14), and to samples of the compounded oil were added 5 parts per million parts of compounded oil of the various polymeric amyl acrylates shown below. The polymers were prepared as shown in Examples 1, 4 and 6. The samples were then stored at a temperature of 25° C. for 15 days. At the end of that time each sample was submitted to the testing procedure described in Example 1 in order to determine the effect of storage on the antifoaming properties of the polymeric amyl acrylate. No foam was observed with samples containing 5 p.p.m. of the following polymers:

Polymeric amyl acrylate,  $CCl_4$  terminated. Mol Wt.=4550

Polymeric amyl acrylate,  $CHCl_3$  terminated. Mol Wt.=5700

Polymeric amyl acrylate, toluene terminated, 10% cyclohexanone. Specific Viscosity=2.13  
Polymeric amyl acrylate, butyl mercaptan terminated. Percent S=0.12

- 5 One of the above samples, i.e., that containing the toluene-terminated polymeric amyl acrylate was again tested at the end of a total of 22 days and then at the end of a total of 60 days storage. No foaming was observed in each case. Blank test samples consisting of only the Champlin 30 base oil or of the same oil to which had been added 4 percent by weight of the detergent additive D-1 had foam values of 710 and 780 cc., respectively at the end of the fifteen-day period.

*Example 16*

- A 30 grade, 93 V.I. base oil was incorporated with 6.5% by weight of an extreme pressure additive comprising chloronaphtha alkyl xanthate (chlorinated naphtha in which only a part of the chlorine has been substituted by an alkyl xanthate group) and a sample of the compounded oil was admixed with a carbon tetrachloride terminated polymeric butyl acrylate in a concentration of 200 parts of polymer per million parts of compounded oil by weight. Evaluation of the foam-susceptibility of the resulting sample employing the testing procedure described in Example 1 showed no foaming after 5 minutes bubbling time, whereas oil containing only the xanthate in absence of the polymer, gave considerable foam when submitted to the same test.

*Example 17*

A 30 grade, 93 V.I. base oil was incorporated with 6.5% by weight of the chloronaphtha alkyl xanthate of

- 60 Example 16 and a sample of the compounded oil was admixed with a normally fluid, carbon tetrachloride terminated polymeric amyl acrylate in a concentration of 100 parts of polymer per million parts of compounded oil by weight. Foaming tests on the resulting sample, employing the procedure described in Example 1, showed no foam at a 5-minute bubbling time.

*Example 18*

- 65 To 93.25 parts by weight of a 30 grade, 93 V.I. oil there was added 6.75 parts by weight of an E.P. additive comprising predominantly the chloronaphtha alkyl xanthate of Example 15 together with minor proportions of an aliphatic dicarboxylic acid ester and an organic phosphate.

The resulting compounded oil showed considerable foaming when submitted to the foaming test described in Example 1. To the compounded oil there was then 75 added the polymeric amyl acrylate of Example 16 in a

concentration equivalent to 100 parts by weight of the polymer per million parts of the finished oil. When the resulting product was submitted to the same foaming test, no foaming was observed at a 5-minute bubbling period.

*Example 19*

Samples of the compounded oils of Examples 16-18, i.e., samples of hydrocarbon oil containing the E.P. additives and the polymeric acrylates were stored for 60 days. No foaming was observed when the stored samples were submitted to the foaming test described in Example 1.

*Example 20*

This example shows the effect of various acrylate-acrylate copolymers on the foaming tendencies of hydrocarbon oils.

The acrylate mixtures shown below were copolymerized in 100 cc. of carbon tetrachloride by maintaining bottles of the solution on a rotating rack (43 r.p.m.) for 48 hours at 98° C. Benzoyl peroxide (1% based on the weight of the monomer mixture) was used as catalyst. The copolymers were recovered by stripping off the solvent, and were incorporated into a Champlin 30 oil in the concentrations shown below. The following foam test data were obtained using the evaluation procedure in Example 1.

| Copolymer Reactants |      |      |          |     |      | Av.<br>Alkyl<br>Chain<br>Length<br>Molar<br>Basis | Foam (cc.) at 5<br>Min. (Copoly-<br>mer, p.p.m.) |     |
|---------------------|------|------|----------|-----|------|---------------------------------------------------|--------------------------------------------------|-----|
| Acrylate            | G.   | Mole | Acrylate | G.  | Mole |                                                   | 40                                               | 10  |
| 2-ethylhexyl        | 24.0 | .130 | Ethyl    | 6   | .060 | 6.1                                               | 0                                                | 0   |
| 2-ethylhexyl        | 21.0 | .114 | Ethyl    | 9   | .090 | 5.4                                               | 0                                                | 0   |
| 2-ethylhexyl        | 24.0 | .130 | Propyl   | 6   | .053 | 6.5                                               | 0                                                | 390 |
| Hexyl               | 25.5 | .164 | Propyl   | 4.5 | .039 | 5.4                                               | 0                                                | 0   |

*Example 21*

A fluid alkyl acrylate-alkyl acrylate copolymer having an average alkyl chain length of 5.35 carbon atoms on a molar basis, and substantially the oil-solubility of amyl acrylate was prepared in kerosene solution as follows:

A mixture consisting of 140 g. of 2-ethylhexyl acrylate, 60 g. of ethyl acrylate, 2 g. of benzoyl peroxide and 800 g. of a kerosene known to the trade as "Skellysolve S" and comprising higher paraffinic hydrocarbons with considerable amounts of aromatics and/or naphthenes, was charged to a reaction vessel equipped with agitator and thermometer, and the mixture was heated to a tempera-

50

This example shows the antifoaming effect of various 2-ethylhexyl acrylate-ethyl acrylate copolymers. The copolymers were prepared in carbon tetrachloride solution and in the presence of about 2 percent of the monomer weight of benzoyl peroxide, polymerization being effected by agitating the solutions at 43 r.p.m. for 65 hours at 80° C. The copolymers were recovered by stripping off the solvent and any unreacted monomer. Foam tests of Champlin SAE 30 oils which had been incorporated with the copolymers were conducted by the method of Example 1. The following results were obtained:

| Copolymer Reactants      |      |                   |      | Av. alkyl<br>chain<br>length<br>molar<br>basis | Mol.<br>Wt. of<br>Co-<br>polymer | Foam (ml.) After 5 Min.<br>(Copolymer in p.p.m.) |     |     |     |     |     |
|--------------------------|------|-------------------|------|------------------------------------------------|----------------------------------|--------------------------------------------------|-----|-----|-----|-----|-----|
| 2-Ethylhexyl<br>acrylate |      | Ethyl<br>acrylate |      |                                                |                                  | 50                                               | 40  | 20  | 10  | 5   | 2   |
| G.                       | Mole | G.                | Mole |                                                |                                  |                                                  |     |     |     |     |     |
| 25.5                     | .139 | 4.5               | .045 | 6.54                                           | 5,460                            | 0                                                | --- | 120 | 450 | 20  | 300 |
| 24.0                     | .130 | 6.0               | .060 | 6.10                                           | 5,340                            | ---                                              | --- | 0   | 20  | 0   | 20  |
| 22.5                     | .122 | 7.5               | .075 | 5.72                                           | 5,280                            | ---                                              | --- | 0   | 0   | 0   | 50  |
| 21.0                     | .114 | 9.0               | .090 | 5.35                                           | 5,520                            | ---                                              | --- | 0   | 0   | 0   | 30  |
| 19.5                     | .106 | 10.5              | .105 | 5.01                                           | 5,660                            | ---                                              | --- | 0   | 10  | 0   | 80  |
| 18.0                     | .098 | 12.0              | .120 | 4.70                                           | 5,660                            | ---                                              | --- | 0   | 25  | 60  | --- |
| 16.5                     | .090 | 13.5              | .135 | 4.40                                           | 5,080                            | 30                                               | --- | 70  | --- | --- | --- |
| 15.0                     | .082 | 15.0              | .150 | 4.12                                           | 4,150                            | 30                                               | --- | 70  | --- | --- | --- |

ture of about 100° C. within one hour. The temperature was maintained at from 97° C. to 102° C. for an additional 5.7 hours. About the middle of the heating period an additional 1-gram portion of benzoyl peroxide was added. At intervals, during the heating period, samples of the reaction mixture were removed in order to note the reaction progress. Refractive index determinations made on the samples showed 54 percent polymerization at the end of 2 hours, 83 percent at the end of 4 hours and 100 percent polymerization at the end of 6.7 hours, at which time heating was discontinued.

70

The above data show that most efficient antifoaming effect is imparted to this oil by copolymers prepared from 65 weight percent to 75 weight percent of the 2-ethylhexyl acrylate and 25-35 weight percent of the ethyl acrylate and having an average alkyl chain length of 5.01 to 5.72.

A similarly prepared polymeric 2-ethylhexyl acrylate gave a foam value of 780 ml. at 50 p.p.m. and a similarly prepared polymeric ethyl acrylate gave a foam value of 705 ml. at the 50 p.p.m. concentration when tested by the same procedure. The base oil had a foam value of 715 ml. in the absence of any additive.

The reaction product, comprising a solution of the 70:30 2-ethylhexyl acrylate-ethyl acrylate copolymer in the kerosene was used directly as an antifoam additive. Incorporation of the solution into a Champlin 30 oil in a quantity corresponding to 10 parts of copolymer per million parts of oil and testing of the treated oil by the method of Example 1 showed no foam at 5 minutes.

*Example 22*

10 A mixture consisting of 210 g. (1.14 moles) of 2-ethylhexyl acrylate, 90 g. (0.9 mole) of ethyl acrylate, 1575 g. of carbon tetrachloride and 5.83 g. (1.94 percent by weight based on total acrylates) was charged to 9 bottles. These were then maintained on a rotating rack at 43 r.p.m. for 40 hours at 95° C. After combining the reaction mixtures the whole was stripped to give 311 g. of the substantially pure, viscous liquid 2-ethylhexyl acrylate-ethyl acrylate copolymer. In order to prepare 15 a concentrate, 150 g. of the liquid copolymer was diluted with 150 g. of toluene and 450 g. of kerosene to give an additive having a 20 percent by weight copolymer content. This was tested with aircraft engine oil 20 as in Example 20. No foam was obtained at a concentration of 10 parts 25 of copolymer per million parts of oil.

## Example 24

This example describes the preparation and usefulness of a 58.3:41.7 (molar ratio) n-octyl acrylate-methyl acrylate copolymer having an average alkyl chain length of 5.07 carbon atoms.

A mixture consisting of 75 g. of n-octyl acrylate, 25 g. of methyl acrylate and 300 g. of a liquid hydrocarbon known as Stoddard Solvent was heated to 100° C. and there were added to the heated mixture four portions of benzoyl peroxide (0.5 g. each) at 45 minute intervals. Heating was continued 45 minutes after the final catalyst addition so that the total heating period at 100° C. was three hours. The reaction mixture, comprising a 25 percent solution of 75:25 (weight ratio) n-octyl acrylate-methyl acrylate copolymer completely inhibited the foaming tendency of a Champlin 30 oil when added to the oil in a concentration equal to 100 parts of additive to a million parts of oil.

## Example 25

Using the procedure of Example 24, there was prepared a 20 percent solution of 48.5:51.5 (molar ratio) decyl acrylate-methyl acrylate copolymer having an average alkyl chain length of 5.37 carbon atoms. The reactants comprised 70.0 g. of decyl acrylate, 30.0 g. of methyl acrylate, 400 g. of Stoddard Solvent and 1.50 g. of benzoyl peroxide. The total heating time at 100° C. was 6 hours.

The reaction product, comprising a solution of a 70:30 (weight ratio) decyl acrylate-methyl acrylate copolymer in the kerosene was used directly as an antifoamant in a 30 grade oil, whereby a quantity corresponding to 100 parts of the copolymer per million parts of oil completely eliminated the foaming tendencies of the oil.

## Example 26

A 29:71 (molar ratio) copolymer of n-lauryl acrylate and ethyl acrylate, having an average chain length of 4.9 carbon atoms, was prepared substantially according to the procedures of Example 24, except that there were used equal parts by weight of the respective acrylates and that a kerosene known to the trade as "Skellysolve S" was used as solvent. The final reaction product comprised a 40 percent solution of the copolymer in "Skellysolve S." When used as an antifoamant in Champlin 30 oil, complete inhibition of the oil to foaming was effected at a concentration of 100 parts of additive to a million parts of oil.

## Example 27

Using the general procedure of Example 24, 60 g. of nonyl acrylate and 40 g. of ethyl acrylate were heated at 100° C. for one hour in 300 g. "Skellysolve S" in the presence of 1.0 g. benzoyl peroxide. After the one hour heating period an additional mixture of 60 g. of nonyl acrylate and 40 g. of ethyl acrylate was gradually added over a period of one hour. Heating at 100° C. was continued for 2 hours with an addition of 0.6 g. benzoyl peroxide every thirty minutes.

The reaction mixture comprising a 40.0 percent solution 60:40 nonyl acrylate-ethyl acrylate copolymer (or 43:57 molar ratio nonyl:ethyl copolymer) having an average alkyl chain length of 5 carbon atoms was used directly as an antifoamant and completely stopped the foaming of a 30 grade oil at a concentration of 100 parts per million.

## Example 28

This example shows the antifoaming effects on Champlin 30 base oil of copolymers of n-butyl or amyl acrylate and styrene. The copolymers were prepared by maintaining bottled solutions of the monomer mixtures for 48 hours on a rotating rack (43 r.p.m.) at a temperature of 90-95° C. In one case the monomer mixture consisted of 27 g. of n-butyl acrylate and 3 g. of styrene and in another experiment the monomer mixture consisted of

25.5 g. of amyl acrylate and 4.5 g. of styrene. In each experiment 100 cc. of carbon tetrachloride was used as solvent and 0.6 g. of benzoyl peroxide was employed as catalyst. The monomers used were employed as received, i.e., without removing any inhibitor present.

In each case reaction mixtures resulting from the polymerization were diluted to 200 cc. with toluene. The diluted materials comprising solutions of the respective copolymers were employed as the antifoam additives. 10 This procedure eliminated the necessity of isolating the polymer (stripping operation) and re-dissolving it in a suitable solvent for use as a concentrate. The quantity of diluted material employed was based on the assumed complete copolymerization of the monomers. Thus, in 15 each case the 200 cc. of toluene-diluted material was assumed to contain 30 g. of copolymer, 0.01 cc. of the diluted material containing 0.0015 g. Accordingly, addition of 0.01 cc. of the diluted material to 37-38 cc. of base oil corresponded to the addition of approximately 20 50 parts of copolymer per million parts of oil. Samples of Champlin 30 base oil which had been thus incorporated with varying amounts of the respective copolymer were tested for foaming as described in Example 1, except that instead of using a 200 cc. sample of oil, 37 cc. 25 of oil was used for each test. No foam was observed at the concentration of 50 parts per million of the respective copolymers; whereas the oil, alone, gave about 70 cc. of foam under the same test conditions.

## Example 29

This example shows the antifoaming effect of copolymers of various alkyl acrylates and acrylonitrile. Employing the copolymerization procedure of Example 28 copolymers were prepared from the following monomer mixtures:

30 27 g. 2-ethylhexyl acrylate and 3 g. acrylonitrile  
27 g. n-butyl acrylate and 3 g. acrylonitrile  
25.5 g. amyl acrylate and 4.5 g. acrylonitrile  
40 Testing of the Champlin 30 base oil as is Example 28 showed no foam for respective test samples containing 50 parts per million of copolymers prepared from the above mixtures.

## Example 30

45 This example shows the antifoaming effect of copolymers prepared from 2-ethylhexyl or n-butyl acrylate and methyl methacrylate. The copolymers were prepared using the polymerization procedure described in Example 28 except that in this instance the following monomer mixtures were used:

50 27 g. 2-ethylhexyl acrylate and 3 g. methyl methacrylate  
25.5 g. 2-ethylhexyl acrylate and 4.5 g. methyl methacrylate  
55 27 g. n-butyl acrylate and 3 g. methyl methacrylate  
27 g. amyl acrylate and 3 g. methyl methacrylate

Copolymers obtained from the above monomer mixtures showed no foaming at 50 parts per million when tested with Champlin 30 base oil as in Example 28.

## Example 31

This example shows the antifoaming effect of copolymers of various acrylates and methacrylonitrile. The polymerization was effected as in Example 28 except that 65 in this instance the following monomer mixtures were used:

60 28.5 g. 2-ethylhexyl acrylate and 1.5 g. methacrylonitrile  
27 g. 2-ethylhexyl acrylate and 3.0 g. methacrylonitrile  
70 27 g. butyl acrylate and 3 g. methacrylonitrile  
27 g. amyl acrylate and 3 g. methacrylonitrile

Addition of the above copolymers, respectively, to Champlin 30 base oil showed no foaming at a concentration of 50 parts per million when tested as in Example 28.

19  
Example 32

This example shows the antifoaming effect of copolymers of various acrylates and vinyl acetate of isopropenyl acetate. The polymerization was effected as in Example 28 except that instead of employing only carbon tetrachloride as solvent, a mixture of 100 cc. of toluene and 100 cc. of carbon tetrachloride was used, and that in this case the following monomer mixtures were used:

24 g. 2-ethylhexyl acrylate and 6 g. vinyl acetate  
21 g. 2-ethylhexyl acrylate and 9 g. vinyl acetate  
27 g. butyl acrylate and 3 g. vinyl acetate  
27 g. amyl acrylate and 3 g. vinyl acetate  
27 g. amyl acrylate and 3 g. isopropenyl acetate

No foaming was observed of Champlin 30 base oil containing 50 parts per million, respectively, of the copolymers obtained from the above mixtures.

## Example 33

Copolymers having the oil-solubility of polybutyl acrylate were prepared by heating for 48 hours at 90-95° C. mixtures of di-n-butyl maleate with n-butyl acrylate or n-amyl acrylate in carbon tetrachloride solution and in the presence of benzoyl peroxide as catalyst. Testing of the antifoaming effect of the copolymers by the test procedure of Example 1 gave the following values:

| Maleate | Reactants Used, g. |          | CCl <sub>4</sub> | Av. Mol. Wt. | Foam (ml.) at 5 Min. (Additive in Parts Per Million of Oil) |    |    |       |       |  |
|---------|--------------------|----------|------------------|--------------|-------------------------------------------------------------|----|----|-------|-------|--|
|         | Acrylate           | Catalyst |                  |              | None<br>710-720                                             | 50 | 10 | 5     | 2     |  |
| 3       | Bu=27              | 1.5      | 154              | 3,450        | -----                                                       | 0  | 10 | ----- | ----- |  |
| 6       | Bu=24              | 1.5      | 154              | 3,070        | -----                                                       | 0  | 10 | ----- | ----- |  |
| 9       | Bu=21              | 1.5      | 154              | 3,130        | -----                                                       | 0  | 10 | ----- | ----- |  |
| 12      | Bu=18              | 1.5      | 154              | 3,130        | -----                                                       | 0  | 0  | 0     | 60-70 |  |
| 15      | Bu=15              | 0.6      | 154              | 4,500        | -----                                                       | 0  | 0  | 20    | ----- |  |
| 12      | Am=18              | 0.6      | 154              | 5,450        | -----                                                       | 0  | 0  | 10    | ----- |  |

## Example 34

This example shows that antifoaming amounts of a liquid 2-ethylhexyl acrylate-ethyl acrylate copolymer have substantially no effect on the viscosity of an oil treated therewith.

A 70:30 2-ethylhexyl acrylate-ethyl acrylate copolymer was prepared as follows: A mixture consisting of 140 g. (0.75 mole) of 2-ethylhexyl acrylate, 60 g. (0.60 mole) of ethyl acrylate, 1050 g. of carbon tetrachloride and 3.89 g. of benzoyl peroxide was charged to 6 bottles, which were then tumbled for 48 hours at 95° C. Removal of solvent from the combined reaction mixtures at 150° C./10 mm. gave 196 g. of the substantially pure 2-ethylhexyl acrylate-ethyl acrylate copolymer having an average molecular weight of 6900 as determined by chlorine analysis of this carbon tetrachloride-terminated product, and an average alkyl chain length of 5.35.

In order to determine if the copolymer caused any appreciable viscosity change in the oil, an untreated sample of a Mid-Continent, solvent-refined SAE grade 10 oil and a sample of the same oil containing 0.05 percent (500 p.p.m.) of the copolymer of this example were prepared, and the viscosity of the specimens determined at 100° F., employing the American Society for Testing Materials method D-445-46T. The untreated oil was found to have a viscosity (S.U.S.) of 207.8, and the value for the treated oil was 207.9. Evaluation of the foam susceptibility of the untreated and treated oil, using the procedure of Example 1 except that instead of using 200 cc. of the oil, 37 cc. of oil was employed for each test, gave a foam of 70 cc. for the untreated oil and no foam for the treated oil. From these data it is apparent that the acrylate-acrylate copolymer confers antifoam property to hydrocarbon oils without causing any appreciable change in the viscosity characteristics of the oil.

45  
50  
55

polymeric alkyl acrylates with that of some polymeric methacrylates.

Employing the polymerization procedure generally described in Example 1, polymerization of monomeric alkyl acrylates or methacrylates was effected in carbon tetrachloride solution to give polymers having the molecular weights shown below. Evaluation of the antifoaming efficiency of the polymers in Champlin 30 base oil, using the evaluation procedure of Example 1 for tests at the 500 p.p.m. concentration, and the procedure of Example 2 for tests at the 50 p.p.m. concentration gave the following results:

| Polymer Additive                   | Foam (cc.) at 5 Min.<br>(Polymer in p.p.m.) |             |
|------------------------------------|---------------------------------------------|-------------|
|                                    | 500                                         | 50          |
| Amyl methacrylate, mol. wt. 5,450  | 950                                         | Over 70 ml. |
| Amyl acrylate, mol. wt. 5,460      | 0                                           | 0.          |
| Hexyl acrylate, mol. wt. 3,130     | 0                                           | 0.          |
| Hexyl methacrylate, mol. wt. 3,100 | 660                                         | Over 70 ml. |

60  
65  
70  
75

This application is a continuation-in-part of my application Serial No. 390,250 filed November 4, 1953, as a continuation-in-part of my application Serial No. 281,680, filed April 10, 1952 and now abandoned.

What is claimed is:

1. A composition of matter of reduced foaming properties consisting essentially of a hydrocarbon oil having foaming tendencies and a quantity less than 0.06% by weight, based on the weight of said oil, said quantity being sufficient to suppress said foaming tendency but insufficient to modify substantially the viscosity characteristics of the oil, of an alkyl acrylate polymer having a molecular weight less than 10,000 and selected from

20  
Example 35

This example shows that antifoaming amounts of a liquid polymeric amyl acrylate have substantially no effect on oil treated therewith. The polymer was prepared as follows:

A mixture consisting of 240 g. of amyl acrylate, 1232 g. of carbon tetrachloride and 4.8 g. of benzoyl peroxide was charged to 8 bottles, and the bottles were maintained on a rotating rack (43 r.p.m.) for 40 hours at 95° C. The reaction mixtures were then combined, and stripped to 160° C./2-3 mm. There was thus obtained as residue 235 g. of the viscous, liquid polymeric amyl acrylate having an average molecular weight of 5250 as determined by chlorine analysis of this carbon tetrachloride-terminated polymer.

A sample of a Mid-Continent solvent-refined SAE grade 10 oil containing 0.05 percent (500 p.p.m.) of the copolymer of this example was tested for viscosity and foaming as in Example 34. The viscosity value of the treated oil was 207.3 (S.U.S.) vs. 207.8 for the oil, alone. The foam test showed no foam for the treated oil, vs. a foam value of 70 ml. for the untreated oil.

## Example 36

This example compares the effect on oil foam of some

the class consisting of (A) a normally fluid homopolymer of an alkyl acrylate having at least 3 but less than 7 carbon atoms in the alkyl radical, (B) a normally fluid copolymer of at least two different alkyl acrylates in which the alkyl radical has from 1 to 18 carbon atoms and in which the average number of carbon atoms in the alkyl radicals of the copolymer molecule is at least 3 but less than 7 on a molar basis and (C) a copolymer having the oil-solubility of (A) and containing at least 50% by weight of an alkyl acrylate in which the alkyl radical has from 1 to 18 carbon atoms with the balance being a compound other than said acrylate and copolymerizable with the acrylate, the said compound being selected from the group consisting of alkyl methacrylates, styrenes, alkyl fumarates, alkyl maleates, alkyl itaconates, acrylonitrile, methacrylonitrile and vinyl esters of aliphatic monocarboxylic acids.

2. A lubricant of reduced foaming properties consisting essentially of a hydrocarbon oil lubricant having foaming tendencies and a quantity less than 0.06% by weight based on the weight of said lubricant, said quantity being sufficient to suppress said foaming tendencies but insufficient to modify substantially the viscosity characteristics of the lubricant, of an alkyl acrylate polymer having a molecular weight in the range from 1513 to less than 10,000 selected from the class consisting of (A) a normally fluid homopolymer of an alkyl acrylate having at least 3 but less than 7 carbon atoms in the alkyl radical, (B) a normally fluid copolymer of two different alkyl acrylates in which the alkyl radical has from 1 to 18 carbon atoms and in which the average number of carbon atoms in the alkyl radicals of the copolymer molecule is at least 3 but less than 7 on a molar basis and (C) a copolymer having the oil-solubility of (A) and containing at least 50% by weight of an alkyl acrylate in which the alkyl radical has from 1 to 18 carbon atoms with the balance being a compound other than said acrylate and copolymerizable with the acrylate, the said compound being selected from the group consisting of alkyl methacrylates, styrenes, alkyl fumarates, alkyl maleates, alkyl itaconates, acrylonitrile, methacrylonitrile and vinyl esters of aliphatic monocarboxylic acids.

3. A detergents hydrocarbon oil lubricant of reduced foaming properties consisting essentially of a hydrocarbon oil lubricant having foaming tendencies and comprising said lubricant, an oil-soluble metal salt as a detergent additive and a quantity less than 0.06 percent by weight of said lubricant, said quantity being sufficient to suppress said foaming tendencies but insufficient to modify substantially the viscosity characteristics of the lubricant, of an alkyl acrylate polymer having a molecular weight less than 10,000 and selected from the class consisting of (A) a normally fluid homopolymer of an alkyl acrylate having at least 3 but less than 7 carbon atoms in the alkyl radical, (B) a normally fluid copolymer of two different alkyl acrylates in which the alkyl radical has from 1 to 18 carbon atoms and in which the average number of carbon atoms in the alkyl radical of the copolymer molecule is at least 3 but less than 7 on a molar basis and (C) a copolymer having the oil-solubility of (A) and containing at least 50% by weight of an alkyl acrylate in which the alkyl radical has from 1 to 18 carbon atoms with the balance being a compound other than said acrylate and copolymerizable with the acrylate, the said compound being selected from the group consisting of alkyl methacrylates, styrenes, alkyl fumarates, alkyl maleates, alkyl itaconates, acrylonitrile, methacrylonitrile and vinyl esters of aliphatic monocarboxylic acids.

4. An extreme pressure-resisting hydrocarbon oil lubricant consisting essentially of a hydrocarbon oil having foaming tendencies, an extreme pressure-resisting additive, and a quantity of less than 0.06 percent by weight based on the weight of said lubricant, said quantity being sufficient to suppress said foaming tendencies but insuffi-

cient to modify substantially the viscosity characteristics of the lubricant, of an alkyl acrylate polymer having a molecular weight less than 10,000 selected from the class consisting of (A) a normally fluid homopolymer of an alkyl acrylate having at least 3 but less than 7 carbon atoms in the alkyl radical, (B) a normally fluid copolymer of two different alkyl acrylates in which the alkyl radical has from 1 to 18 carbon atoms and in which the average number of carbon atoms in the alkyl radical of the copolymer molecule is at least 3 but less than 7 on a molar basis and (C) a copolymer having the oil-solubility of (A) and containing at least 50% by weight of an alkyl acrylate in which the alkyl radical has from 1 to 18 carbon atoms with the balance being a compound other than said acrylate and copolymerizable with the acrylate, the said compound being selected from the group consisting of alkyl methacrylates, styrenes, alkyl fumarates, alkyl maleates, alkyl itaconates, acrylonitrile, methacrylonitrile and vinyl esters of aliphatic monocarboxylic acids.

5. A lubricant of reduced foaming properties consisting essentially of a hydrocarbon oil lubricant having foaming tendencies and a quantity of less than 0.06 percent by weight, based on the weight of said lubricant, said quantity being sufficient to suppress said foaming tendencies but insufficient to modify substantially the viscosity characteristics of the lubricant, of a normally fluid homopolymer of an alkyl acrylate having at least 3 but less than 7 carbon atoms in the alkyl radical and the homopolymer having a molecular weight less than 10,000.

6. A lubricant of reduced foaming properties consisting essentially of a hydrocarbon oil lubricant having foaming tendencies and a quantity of less than 0.06 percent by weight, based on the weight of said lubricant, said quantity being sufficient to suppress said foaming tendencies but insufficient to modify substantially the viscosity characteristics of the lubricant, of a normally fluid copolymer of two different alkyl acrylates in which the alkyl radical has from 1 to 18 carbon atoms and in which the average number of carbon atoms in the alkyl radical of the copolymer molecule is at least 3 but less than 7 on a molar basis, the copolymer having a molecular weight less than 10,000.

7. A lubricant of reduced foaming properties consisting essentially of a hydrocarbon oil lubricant having foaming tendencies and a quantity of less than 0.06 percent by weight based on the weight of said lubricant, said quantity being sufficient to suppress said foaming tendencies but insufficient to modify substantially the viscosity characteristics of the lubricant of a copolymer possessing the oil-solubility of a normally fluid homopolymer of an alkyl acrylate having at least 3 but less than 7 carbon atoms in the alkyl radical, said copolymer containing at least 50% by weight of an alkyl acrylate in which the alkyl radical has from 1 to 18 carbon atoms with the balance being a compound other than the acrylate and copolymerizable with the acrylate, the said compound being selected from the group consisting of alkyl methacrylates, styrenes, alkyl fumarates, alkyl maleates, alkyl itaconates, acrylonitrile, methacrylonitrile and vinyl esters of aliphatic monocarboxylic acids and said copolymer having a molecular weight less than 10,000.

8. The lubricant of claim 5 further defined in that said polymer is a normally fluid polymeric butyl acrylate.

9. The lubricant of claim 5 further defined in that said polymer is a normally fluid polymeric amyl acrylate.

10. The lubricant of claim 7 further defined in that said polymer is a normally fluid copolymer of 2-ethylhexyl acrylate and acrylonitrile consisting, by weight, of from 85% to 90% of copolymerized 2-ethylhexyl acrylate and 10% to 15% of copolymerized acrylonitrile.

11. The lubricant of claim 7 further defined in that said polymer is a normally fluid copolymer of 2-ethylhexyl acrylate and methyl methacrylate consisting, by weight, of from 80% to 90% of copolymerized 2-ethylhexyl

acrylate and from 10% to 20% of copolymerized methyl methacrylate.

12. The lubricant of claim 1 further defined in that the molecular weight of the polymer is no greater than 6900.

13. The lubricant of claim 6 further defined in that the average number of carbon atoms in the alkyl radical of the copolymer molecule is in the range of 4.5 to 6 and the molecular weight of the copolymer is in the range of 5 3100 to no greater than 6900.

14. The lubricant of claim 13 further defined in that 10 the quantity of the copolymer is less than 0.01% by weight, based on the weight of said lubricant.

15. The lubricant of claim 5 further defined in that the alkyl acrylate has 5 to 6 carbon atoms in the alkyl radical and a molecular weight of from 1513 to less than 15 10,000.

16. A lubricant of reduced foaming properties consisting essentially of a hydrocarbon oil lubricant having

foaming tendencies and a quantity less than 0.1% by weight based on the weight of said lubricant, said quantity being sufficient to suppress said foaming tendencies but insufficient to modify substantially the viscosity characteristics of the lubricant, of a normally fluid copolymer of 2-ethylhexyl acrylate and ethyl acrylate consisting, by weight, of from 65% to 75% of copolymerized 2-ethylhexyl acrylate and 25% to 35% of copolymerized ethyl acrylate.

#### References Cited by the Examiner

##### UNITED STATES PATENTS

|           |       |                  |        |
|-----------|-------|------------------|--------|
| 2,330,773 | 9/43  | Zimmer           | 252-56 |
| 2,430,858 | 11/47 | Borsoff et al.   | 252-52 |
| 2,600,448 | 6/52  | Van Horne et al. | 252-56 |
| 2,604,453 | 7/52  | Popkin           | 252-56 |

DANIEL E. WYMAN, Primary Examiner.